

## UNITED STATES PATENT OFFICE

2,488,513

## PRODUCTION OF WHITE CAST IRON

Henton Morrogh, Handsworth, England, assignor  
to British Cast Iron Research Association,  
Alvechurch, England

No Drawing. Application February 4, 1949, Serial No. 74,709. In Great Britain February 10, 1948

6 Claims. (Cl. 75—123)

1

This invention relates to the production of white cast iron in a form specially suitable for subsequent annealing.

In white cast irons as normally produced for annealing (e. g. to give malleable cast iron) the whole of the carbon content is present as iron carbide (cementite), which gives to the white iron its hardness and brittleness. In order to reduce this brittleness it is customary to subject the cast iron to a heat treatment at high temperatures (800–1000° C.) for lengthy periods (20 to 200 hours) in order to decompose the cementite. The carbon liberated during this annealing process appears in the form of graphite nodules distributed throughout the metal. The decomposition of cementite by heat is facilitated by the presence of silicon, and the lower annealing times and/or temperatures above mentioned are applicable to white irons rich in silicon. The higher the silicon content, however, the more likely is the cast iron to be grey instead of white. In grey cast iron the carbon is present wholly or in part as flake graphite which renders it useless for the production of malleable iron. Even high-silicon irons, however give a white cast iron in the presence of a sufficiency of cerium or tellurium.

In relation to their carbon content cast irons may be eutectic, hypereutectic or hypo-eutectic. The carbon content in a eutectic iron varies with the silicon and phosphorus contents, and corresponds sufficiently accurately for present purposes with the formula

$$C = 4.3 - \frac{1}{3}(P + Si)$$

where C, P and Si stand for the percentages of carbon, phosphorus and silicon, respectively. If the percentage of carbon in the cast iron is greater than is given by this formula, the iron is said to be hypereutectic; if less, hypo-eutectic.

It is an object of the present invention to produce a readily annealable white cast iron. It is a further object to produce such a cast iron from hypereutectic irons. A still further object is to produce a white cast iron in which the hypereutectic carbon (i. e. the excess of carbon over the eutectic proportion) is present in the form of nodular graphite. Other objects will appear from the following description.

I have found that the addition of cerium to a hypereutectic iron before casting results, provided the iron is low in sulphur and phosphorus, in a cast iron in which the hypereutectic carbon is wholly or preponderantly in the form of nodular

2

graphite. The structure comprises a fine dispersion of graphite nodules in an otherwise white iron. I have found that the presence of these nodules greatly facilitates the subsequent annealing process, decomposition of the cementite taking place at lower temperatures and/or in shorter times than have hitherto been found necessary.

According to the invention, therefore, cerium is added to a hypereutectic iron which on casting gives a cast iron containing not more than 0.02% of sulphur, less than 0.5% of phosphorus, and not more than 7% of silicon, so as to yield a white cast iron in which the hypereutectic carbon is wholly or preponderantly in the form of nodular graphite.

Cerium is a powerful desulphurising agent but economic considerations make it necessary to use as starting material an iron already low in sulphur and not to use up valuable cerium in reducing the sulphur content to the required limit. Any cerium sulphide present in the cast iron is entirely ineffective in the production of nodular graphite. If the starting material contains too much sulphur it should be pretreated with one of the known and cheaper desulphurising agents.

The amount of cerium to be added must be sufficient to give a white cast iron. With section sizes of one inch or less, 0.02 to 0.08% of cerium in the cast iron will be found satisfactory. (By "section size" is meant the diameter of the casting at its narrowest part). This is due to the more rapid cooling of the smaller sections, and a corresponding effect is obtained by the use of a metal or chill mould in comparison with a sand mould.

Rapid cooling of the casting also enables white iron castings to be made from iron containing the higher proportions (up to the limit of 7%) of silicon.

The smaller the section size and the greater the cooling rate, the higher may be the silicon content and the lower the amount of cerium required.

Up to 5% of cerium may be used if desired, but owing to the cost of this metal and, as explained below, the longer time and/or higher temperatures required for annealing when much cerium is present, I prefer to limit the cerium to not more than 0.2% in the cast iron.

The annealing of castings produced according to the invention requires much less time than in the case of ordinary white cast iron. The time of heating will vary according to the content of cerium and, as already indicated, of silicon. Longer periods and/or higher temperatures are needed according as the cerium content is higher and/or the silicon content lower.

## 3

In order to assist the deposition of the hypereutectic carbon in the form of graphite (which in the presence of the cerium appears as nodules instead of flakes), it is advantageous to add a graphitising inoculant, such as ferrosilicon, calcium silicide, graphite itself, or mixtures of any or all of these. The addition should be made after the cerium has been added and immediately before pouring the molten iron. This treatment increases the number of hypereutectic nodules and hence the rate of subsequent graphitisation. The nature of the invention will be understood from the following illustrative example, in which, as elsewhere in the description and claims, percentages are by weight.

## Example

Fifty pounds of pig iron of the composition:

|                 | Per cent |
|-----------------|----------|
| Total carbon    | 3.80     |
| Silicon         | 2.69     |
| Manganese       | 0.66     |
| Sulphur         | 0.030    |
| Phosphorus      | 0.045    |
| Iron, remainder |          |

was melted in a crucible furnace. To the molten metal were added first  $2\frac{1}{2}$  oz. of mischmetall and then 4 oz. of 80% ferrosilicon. The metal was poured into cold graphite chill moulds giving test bars 0.875 inch diameter. A test bar showed on analysis:

|                 | Per cent |
|-----------------|----------|
| Total carbon    | 3.66     |
| Silicon         | 2.96     |
| Manganese       | 0.60     |
| Sulphur         | 0.017    |
| Phosphorus      | 0.044    |
| Cerium          | 0.051    |
| Iron, remainder |          |

The microstructure of these as-cast bars consisted of dispersed nodules of graphite in a white cast iron matrix.

The bars were annealed by heating at 950° C. for 35 minutes and allowing to cool to room temperature in 5 hours. The microstructure of the annealed bars consisted of uniformly distributed graphite nodules in a matrix of ferrite. The mechanical properties (average of three closely concordant results) were:

Ultimate tensile strength \_\_\_\_ tons/sq. in. 25.6  
Elongation at break \_\_\_\_ per cent 6.5

It will be seen that the invention provides a cast iron which can be economically annealed. It is applicable to the production not only of

## 4

malleable cast iron but also of die-castings which are to be annealed. For malleable cast iron a sand mould is usually employed and accordingly the silicon content should be low rather than high. For castings in dies or permanent moulds (chill castings) there is no objection to higher silicon content within the limit of 7% above specified.

I claim:

10 1. A white cast iron containing 0.02 to 5.0% of cerium, not more than 0.02% of sulphur, less than 0.5% of phosphorus and not more than 7% of silicon, and having a carbon content greater than

$$15 4.3 - \frac{1}{3}(P + Si)$$

where P and Si stand for the percentages of phosphorus and silicon, respectively, in the cast iron, the hypereutectic carbon content being preponderantly in the form of nodular graphite.

20 2. A white cast iron as claimed in claim 1 which has been subjected to an annealing process.

25 3. Process for the production of white cast iron especially suitable for annealing, comprising adding to an iron which is hypereutectic in relation to carbon and which after casting contains not more than 0.02% of sulphur, less than 0.5% of phosphorus and not more than 7% of silicon such an amount of cerium as will result in a white iron casting containing 0.02 to 5.0% of cerium (other than that present as cerium sulphide).

30 4. Process as claimed in claim 3 in which the amount of cerium added is such as will result in a white iron casting containing 0.02 to 0.2% of cerium (other than that present as cerium sulphide).

35 5. Process for the production of white cast iron especially suitable for annealing, comprising adding to an iron which is hypereutectic in relation to carbon and which after casting contains not more than 0.02% of sulphur, less than 0.5% of phosphorus and not more than 7% of silicon such an amount of cerium as will result in a white iron casting containing 0.02 to 5.0% of cerium (other than that present as cerium sulphide) and, after the addition of the cerium and immediately before casting, adding a graphitising inoculant.

40 6. Process as claimed in claim 5 in which the graphitising inoculant is selected from the group consisting of ferrosilicon, calcium silicide, graphite, and mixtures of at least two of these substances.

HENTON MORROGH.

No references cited.